

Sept. 15, 1936.

W. FORSTMANN

2,054,284

PHOTOGRAPHIC FILM

Filed May 31, 1933



Inventor:  
Walther Forstmann  
by *Karl Schickhardt*  
Atty.

## UNITED STATES PATENT OFFICE

2,054,284

## PHOTOGRAPHIC FILM

Walther Forstmann, Berlin-Schöneberg, Germany, assignor to Voigtlander & Sohn Aktiengesellschaft, Brunswick, Germany

Application May 31, 1933, Serial No. 673,599½  
In Germany June 6, 1932

5 Claims. (Cl. 95—9)

My invention relates to photographic films, more especially of the kind in which an intermediate substratum layer is inserted between the sensitive layer and the film body serving as 5 carrier of this sensitive layer.

It is an object of my invention to provide a film comprising such an intermediate layer which is superior to similar layers hitherto used as far as the power to hold the sensitive layer on the 10 carrier is concerned.

As is well known to those skilled in the art, a gelatine layer as constituted by a photographic emulsion, when arranged directly on a base or carrier such as cellulose nitrate, cellulose acetate 15 or the like, will not adhere to this carrier as solidly as required in practical use. After the gelatine has dried down on the carrier, it can as a rule be stripped as a whole, and on being acted upon by a watery liquid, such as a developer, fixation or reinforcing liquor, the gelatine 20 layer will frequently come off, starting from the edges.

In order to improve the adhesion of the sensitive layer to the carrier or film body an intermediate layer serving as binder has been inserted between the two parts. To this end carriers consisting of nitrocellulose have been coated with a preparation consisting of gelatine pre-treated by allowing it to swell in small quantities of water, dissolving the swollen gelatine by 25 adding glacial acetic acid and diluting the gelatine solution with alcohol, acetone or the like.

In the case of cellulose acetate films a preparation has been applied containing, besides gelatine, acetic acid and alcohol, also small quantities of nitrocellulose, however the adhesive properties of a sensitive layer fixed to the film by means of this preparation have frequently been found to be unsatisfactory, since the 30 physical properties of the cellulose acetate vary from batch to batch.

In the case of films prepared from certain kinds of diacetates and more especially triacetates and mixed cellulose acetate esters the 35 preparations described above are an absolute failure, for, while the gelatine or emulsion may adhere firmly to the intermediate layer formed of such preparation, the cohesion between the intermediate layer itself and the film body is not a satisfactory one.

I have now found that a perfect adhesion can be attained provided that the solution from which the intermediate or binding layer is produced, contains as a constituent a certain proportion 50 of the material constituting the film body, i. e.

the same or a similar cellulose derivative, or some of the cotton product used in the preparation of the body material.

While it appears impossible, at the present time, to account with any degree of certainty for the 5 increase in the adhesive power, which is thus attained, an explanation which appears to offer itself by way of suggestion, is that the more or less finely dispersed gelatine particles, when drying, are cemented to the film body by the dry- 10 cellulose ester admixed to the gelatine. Probably cellulose compounds of a different type, such as the nitrocellulose previously suggested as a constituent of such intermediate layer, are not capable of adhering to the surface of the 15 cellulose ester film body as firmly as a layer containing the same ester or the cotton, from which it is prepared.

By adding to the intermediate layer some of the film body material, I obtain the further advantage that the quantity of solvents liable to attack the film body material and to cause warping of the film, can be reduced considerably. I am further enabled to dispense with the addition 20 of stronger acids such as the acetic acid, which 25 is very desirable from a photographic standpoint, for, when the intermediate layer dries down, the acetic acid present therein will not evaporate altogether and the traces of acid remaining over in the emulsion will cause a reduction of the 30 storing capacity and the resistance against the influence of higher temperatures (in hot climates), the emulsion being liable to become foggy and less sensitive to light.

In the accompanying drawing I have, without 35 restricting my invention thereto, shown by way of example a film embodying my invention, the view being a conventional exaggerated cross-sectional showing.

In practicing my invention, I may for instance 40 proceed as follows:

I allow 10 parts by weight gelatine to swell in 30 parts water, in which 5 parts salicylic acid are dissolved, and I then add a solution of 10 parts of the film body material such as for instance cellulose triacetate in 800 parts acetone, 1000 parts ethanol and 1200 parts methylene chloride.

This solution is poured for instance on a cellulose triacetate film containing tricresyl phosphate 50 and other softening agents. After the solvents have been evaporated, the emulsion is poured on the intermediate layer thus formed.

The percentage of film material or cotton to be dissolved in the solution designed to form the 55

intermediate layer depends from the physical and chemical properties of the body material and the character and thickness of the hydrophil colloid layer (for instance the photographic emulsion) 5 to be subsequently deposited on the intermediate layer. It may vary for instance between one-tenth of and three times the quantity of gelatine incorporated in the intermediate layer.

This layer has been found to firmly cement the 10 emulsion to the film body.

I have found that I may obtain a similar effect, when incorporating in the solution forming the intermediate layer a cellulose compound or cotton of the same type, however possessing physical 15 properties differing from those of the film body material. For instance in the case of a film formed from highly viscous cellulose triacetate, I may use an intermediate layer containing a low viscosity triacetate or a mixture thereof with the 20 same high viscosity material.

Obviously my invention is not limited to intermediate layers formed with gelatine, but is applicable also to layers containing any other kind of colloids of similar action, including agar-agar, 25 isinglass, albumen etc.

Of the hydrophil colloids which may be spread on the intermediate layer, I may mention, besides gelatine and photographic emulsion, also agar-agar, albumen, gum arabic etc. and mixtures of 30 two or more of these substances.

It is however not necessary that the colloids contained in the intermediate layer and the superposed layer (sensitive layer) be identical, and I may for instance pour an agar-agar solution 35 on an intermediate layer formed with gelatine.

Various changes may be made in the details disclosed in the foregoing specification without departing from the invention or sacrificing the 40 advantages thereof.

I claim:—

1. Photographic film comprising in combination, a film body containing a cellulose ester, a

sensitized layer, and an intermediate substratum layer inserted between, and inter-united with, said film body and said sensitized layer and being a substantially homogeneous mixture of a hydrophil colloid and a cellulose ester of the same chemical composition as the said cellulose ester contained in said film body. 5

2. Photographic film comprising in combination, a film body containing a cellulose ester, a sensitized layer and an intermediate substratum 10 layer inserted between said film body and said sensitized layer and being a substantially homogeneous mixture of a hydrophil colloid and the same cellulose ester as said film and which is interunited with said film and with said sensitized 15 layer.

3. Photographic film comprising in combination, a cellulose acetate film body, an intermediate substratum layer on said film body being a substantially homogeneous mixture of cellulose acetate and a hydrophil colloid, and a sensitized layer on said intermediate layer, the said substratum layer being inter-united with said film body and with said sensitized layer. 20

4. Photographic film comprising in combination, a film body containing a cellulose ester, a sensitized layer and an intermediate substratum layer inserted between said film body and said sensitized layer and being a substantially homogeneous mixture of a hydrophil colloid and from one-tenth to the treble, calculated on this colloid, of a cellulose ester containing the same acid radical as said cellulose ester contained in 25 said film body. 30

5. Photographic film comprising in combination, a film body containing a mixed cellulose acetate ester, a sensitized layer, and an intermediate substratum layer inserted between, and inter-united with, said film body and said sensitized layer and being a substantially homogeneous 40 mixture of a hydrophil colloid and a cellulose ester of the same acid as the film body. 35

WALTHER FORSTMANN.